

Patented Nov. 17, 1925.

1,562,043

# UNITED STATES PATENT OFFICE.

ALADAR PACZ, OF EAST CLEVELAND, OHIO, ASSIGNOR TO GENERAL ELECTRIC COMPANY, A CORPORATION OF NEW YORK.

## IRON-BORON ALLOY.

No Drawing.

Application filed March 7, 1922. Serial No. 541,837.

*To all whom it may concern:*

Be it known that I, ALADAR PACZ, a citizen of the United States, residing at East Cleveland, in the county of Cuyahoga, 5 State of Ohio, have invented certain new and useful Improvements in Iron-Boron Alloys, of which the following is a specification.

My invention relates to metals for casting and more specifically to such metals consisting principally of iron. The object of my invention is to provide a metal which will possess the good casting qualities of cast iron and at the same time possess higher tensile strength, greater homogeneity and better adaptability for working than cast iron.

My invention consists in incorporating with the iron a small percentage of boron. 20 Although there are disclosures in the prior art of the use of boron in connection with iron and steel, they have had little effect on the iron and steel industry. I believe that I am the first to recognize in the combination of boron with iron, the especial advantages for casting which it possesses over cast steel, and, at the same time, the higher tensile strength and workability which it possesses over cast iron.

My invention provides a metal which has a higher tensile strength than that of cast iron and even higher than those of semi-steel or malleable cast iron. It machines like soft cast iron and more easily than steel because of its lack of ductility as cast. On the other hand, it may be forged and drawn since it acquires ductility by working. Its low melting point, which may be varied by the addition of greater or lesser 40 percentages of boron, and which in some cases is lower than that of cast iron, is of great advantage on account of greater fluidity of the molten metal and also less shrinkage of castings. On account of its higher tensile strength, articles can be made

of smaller dimensions than if cast iron were employed. Another feature of my invention is that the castings made from this metal do not chill, and therefore the metal is particularly adaptable for casting in metal molds. On account of its comparatively fine grained structure and uniformity, with absence of blow-holes, the metal does not warp like cast iron, nor is it so porous. The use of my metal for castings

reduces the number of rejections on account of defects as compared with cast iron. When machined, the metal takes a very smooth finish. The elasticity is much higher than that of cast iron.

The above stated properties render my metal especially suitable for piston rings, pistons, engine valves, cylinders for internal combustion and other engines, molds, dies, pump parts, and many of the other uses 65 to which cast iron and cast steel are now put.

I have found it desirable to incorporate about from three-fourths per cent to four per cent of boron in the iron. Above 4 70 per cent the cost is rather high and the hardness and brittleness are too high for ordinary purposes. One alloy which I have found to be very serviceable contained about from one and six-tenths per cent to two per 75 cent of boron. This was made by adding to ninety pounds of low carbon steel scrap, having about one-tenth per cent carbon, ten pounds of ferro-boron, containing from sixteen to twenty per cent of boron. The percentage of carbon in the steel scrap is important because the hardness of the final product will depend largely upon its carbon content. The ferro-boron which I prefer to use is that produced by the aluminothermic method, as set forth in my application, Serial No. 294,456, filed May 3, 1919, although I do not restrict myself to this source of boron. The metal produced with the above stated proportions of materials 80 had a melting point slightly higher than that of cast iron. It had a tensile strength of from sixty-seven thousand pounds per square inch. It was forged at a red heat and this raised the tensile strength to 95 about one hundred five thousand pounds per square inch with an elongation of six per cent.

Tensile strengths upwards of fifty thousand pounds may be readily obtained 100 through my invention. The carbon content may vary although I prefer to have less than one-half per cent carbon present.

What I claim as new and desire to secure by Letters Patent of the United States, is:

1. A casting, consisting predominantly of iron with from three-fourths to four per cent of boron, and having a tensile strength upwards of fifty thousand pounds per square inch.

2. A chilled casting, consisting predominantly of iron, with from three-fourths to four per cent of boron, and having a tensile strength upwards of fifty thousand pounds per square inch.
3. A cast alloy having a tensile strength upwards of fifty-thousand pounds per square inch and consisting predominantly of iron, less than one-half per cent carbon, and three-fourths to four per cent boron.
4. A cast piston ring composed of an alloy containing mostly iron, with three-fourths to four per cent boron.
5. A cast piston ring composed of an alloy containing mostly iron, with three-fourths to four per cent boron, and less than one-half per cent carbon.

In witness whereof, I have hereunto set my hand this 3rd day of March 1922.

ALADAR PACZ.